

## UNITED STATES PATENT OFFICE

BORIS N. LOUGOVY, OF MONTCLAIR, NEW JERSEY, ASSIGNOR TO ELLIS-FOSTER COMPANY, OF MONTCLAIR, NEW JERSEY, A CORPORATION OF NEW JERSEY

## LACQUER AND LACQUER ENAMEL CONTAINING CERTAIN PETROLEUM PRODUCTS

No Drawing.

Application filed November 16, 1925. Serial No. 69,502.

This invention relates to a coating composition containing cellulose ethers or esters, and relates particularly to nitrocellulose solutions adapted for use as lacquers or lacquer enamels.

5 The composition of the present invention in its preferred form comprises nitrocellulose, with or without other solid material, such as natural or synthetic resins, with or without 55 out pigments, carried in a vehicle comprising a petroleum distillate boiling preferably above 100° C., but preferably not exceeding about 150° C.; said distillate preferably containing some unsaturated hydro carbons de- 60 rived by cracking operations.

10 As a true solvent for the nitrocellulose I prefer to use one which does not possess excessive volatility, and find butyl acetate desirable for the purpose.

20 While butyl acetate dissolves nitrocellulose readily, it does not permit of a considerable addition of the petroleum hydrocarbon fraction referred to above without yielding cloudy films. These are not desirable 25 when transparent effects are required, and even when pigments are used, the fact that the film is of a turbid character leads to the suspicion that it is not homogeneous, and therefore, that its durability as a coating will 30 not prove satisfactory.

25 Petroleum distillates having very low boiling points, as, for example, 50° C., are usually inappropriate, at least if present in any quantity, in producing the composition of the present invention. On the other hand, distillates boiling above 200° C., as a rule are 35 too heavy, remaining in the film exposed to evaporation for a period longer than that of the nitrocellulose solvents, and causing precipitation. Above 50° C., and preferably 40 below 200° C., therefore, constitutes what may be termed approximately the limiting range of boiling points. However, I prefer a distillate with a more restricted range than 45 the foregoing, as, for example, I may use one boiling between 100° C., and 135° C., e. g., this fraction from a distillate obtained by cracking petroleum under several atmospheres pressure. A more desirable distillate 50 is that boiling between 120° C., or 130° C.,

up to 150° C., or 160° C. In general by employing a distillate having a boiling point range not greater than 30-35° C., desirable results may be secured in the practice of my invention. For example, a distillate whose lower boiling point is 125° C., may have an upper boiling point of approximately 155-160° C. By confining the distillate, especially one containing cracked petroleum, within such specified limiting boiling points, I obtain very useful effects.

55 In the manufacture of lacquer enamels which are to be applied by spraying devices, I may use such restricted boiling point distillates to advantage.

60 The effect of using such narrow range petroleum distillates with nitrocellulose gives rise to certain unexpected results. Using an effective nitrocellulose solvent, for example, butyl acetate, which I prefer, and adding narrow range boiling point petroleum distillate to a solution of soluble cotton in butyl acetate, it is possible to add the distillate in at least an equal volume without producing a cloudy solution. On pouring out such a 65 solution onto a flat surface and allowing the coating to dry, a cloudy or opaque film is likely to result. I have discovered, however, that the addition of a small amount of a third solvent, such as butyl alcohol, or diacetone alcohol, will overcome this cloudiness, yielding a clear brilliant film. The proportion of the butyl alcohol (butanol) required, is surprisingly small, ordinarily three to five 70 per cent of the clarifying agent being sufficient to accomplish the desired result.

75 In one case I prepared from petroleum products a distillate whose boiling point range was between the narrow limits of 130 and 150° C. Such a product was obtained by the 80 fractionation of a hydrocarbon mixture containing both straight-run gasoline and pressure cracked gasoline, and therefore having cyclic bodies and unsaturated compounds, the presence of which I consider desirable in preparing compositions in accordance with the 85 present invention.

90 A twenty per cent solution of low viscosity soluble cotton (what is known as one-half second cotton) was prepared with butyl ace- 95

55

60

65

70

75

80

85

90

95

100

tate as the solvent. I found that this solution could be diluted with the above narrow-range boiling-point petroleum fraction to the extent of equal volumes, or even six parts of the petroleum fraction to five parts of the butyl acetate solution, without causing any precipitation of the nitro cotton. One composition was made having the proportion of one part of nitro cotton, five parts of butyl acetate, and six parts of petroleum distillate. The solution was clear, but on evaporation, an opaque white film, considered valueless from the coating standpoint, was obtained. It was found, however, most surprisingly, that this film could be rendered transparent when dry, if a few per cent of certain solvents were added to the solution. Thus, four or five per cent of primary butyl alcohol, or commercial butanol, diacetone alcohol, or amyl alcohol, were found to serve as effective clarifiers.

When resins, which are frequently required in lacquer enamels to give adhesion, are present, the difficulties of making a clear film increase. Many resins are not soluble in such petroleum distillates. This is especially true of a number of synthetic resins, such as those prepared from glycerine and organic acids. Certain natural resins, such as damar or shellac, are not readily soluble in petroleum distillates.

By employing cracked distillate of appropriate boiling point spread, with or without straight run distillate, I am able to employ many of these resins despite their very great variation in solubility characteristics.

My invention is especially useful in the case of low viscosity nitro cotton. The employment of cracked petroleum distillate with such low viscosity cotton is most advantageous and affords a solvent mixture of novel characteristics and of surprising effectiveness. Furthermore, the use of so-called alcohol-soluble nitro cotton is not precluded. The invention in one phase, therefore, embraces a coating composition comprising such low viscosity nitro cotton, a solvent therefor, and a cracked petroleum distillate, having a boiling point range preferably within the general limits indicated.

While I have specified a distillate having a boiling point "spread" of 30° to 35° C., I do not wish to be limited to this in all cases but may use a fraction boiling between 100 and 150° C., thus having a spread of 50°, or in some cases, may increase the spread to a greater extent, preferably avoiding the highly volatile low fractions of excessive inflammability with consequent fire hazard, e. g., below 40° or 50° C. In such low fractions also there may be present unsaturated bodies which resinify on exposure, forming products incompatible with nitrocellulose, which is disadvantageous.

In making lacquers, when employing such

petroleum distillates, especially those containing cracked material, it is recommended that the pigment employed be ground with the nitrocellulose solution containing the petroleum distillate; employing a ball mill, or similar effective grinding means, and continuing the grinding until the pigment reaches a state of fineness or dispersion such that the distillate does not tend to bring about pigment-coagulation when the exposed coating dries.

What I claim is:—

1. A coating composition capable of yielding a clear film on evaporation, comprising low viscosity nitrocellulose, a solvent therefor, and a substantial proportion of a petroleum distillate, comprising cracked petroleum, and having a boiling point range between 100° C., and 200° C; the highest boiling component having a boiling point not exceeding the lowest boiling point component thereof by more than 35° C.

2. A coating composition comprising a solution of nitrocellulose in a volatile solvent vehicle comprising a substantial proportion of a petroleum distillate boiling between 130° C., and 150° C., and containing a clarifying agent; whereby clear films are obtained on evaporation.

3. A liquid coating composition comprising nitrocellulose, butyl acetate and a petroleum distillate, boiling between 100 and 150° C.

4. A composition comprising nitrocellulose, a solvent and a petroleum distillate boiling between 100 and 150° C., which contains unsaturated hydrocarbons derived from cracking operations.

5. A coating composition comprising nitrocellulose, butyl acetate and a distillate from cracked petroleum, said distillate having a boiling point between 125 and 160° C.

6. A coating composition comprising nitrocellulose, a solvent, a petroleum distillate boiling between 100 and 150° C., and containing unsaturated hydrocarbons derived from cracking operations, and an alcohol containing clarifier.

7. A coating composition comprising nitrocellulose, a solvent therefore, and a distillate, boiling between 100 and 135° C., derived from pressure cracked petroleum.

8. A liquid coating composition comprising nitrocellulose, a solvent therefor, and a distillate boiling between 130 and 150° C., obtained from a hydrocarbon mixture containing both straight run and pressure cracked gasoline.

9. A liquid coating composition comprising low viscosity nitrocellulose, butyl acetate and a petroleum distillate boiling between 100 and 150° C.

10. A liquid coating composition comprising nitrocellulose, a solvent therefor, and a petroleum distillate, boiling between 100 and

150° C., and containing unsaturated hydrocarbons derived from cracking operations, and a resin.

11. A liquid coating composition comprising nitrocellulose, a solvent therefor, a petroleum distillate boiling between 100 and 150° C., and containing unsaturated hydrocarbons derived from cracking operations, and a synthetic resin.

10 12. A liquid coating composition comprising nitrocellulose, a solvent therefor, and a petroleum distillate boiling between 100 and 150° C.

BORIS N. LOUGOVOY.

15

20

25

30

35

40

45

50

55

60